

## UNITED STATES PATENT OFFICE

2,008,939

METHOD OF AND MATERIAL FOR  
TREATING METAL

John L. Tufts, Worcester, Mass.

No Drawing. Application July 29, 1932,  
Serial No. 626,211

18 Claims. (Cl. 205—21)

This invention relates to a method of and material for treating metal, and more specifically relates to lubricating and cold-working metal, removing the lubricant by a simple water rinse, 5 and applying a permanent finishing coat, and to a lubricating material suitable for use in carrying out this method.

The permanent finishing coat referred to may be paint, lacquer, enamel, electro-plating or other 10 applied coat, or a phosphate or other chemically formed coat.

In cold-working processes, such as machining, drawing, punching, stamping, etc., it has been customary to lubricate the metal with oil, grease 15 or emulsions thereof. Such a lubricant must be very thoroughly removed before finishing the surface with a permanent coat or remnants of the oil or grease will interfere with the proper formation or binding of the coat. A simple water rinse 20 does not remove the greasy lubricant, and proper cleaning involves considerable expense and requires careful work. The metal surface may appear bright and clean while retaining sufficient residual grease to interfere with proper finishing. 25

A careful workman may detect such imperfect cleaning by observing what is known as "water break," that is, when water draining from the surface leaves drops or spots instead of an evenly distributed thin film of water on the surface; but hurried or careless work may easily result in imperfect cleaning and consequently inferiority in 30 the finished product.

It may be noted incidentally that ordinary lubricating materials frequently contain substances 35 which may produce insoluble greasy metal soap deposits, that increase scouring difficulty.

On the other hand, where metal working treatment is done according to the present invention, metal products free from "water break" are quickly 40 available by a simple water rinse.

This ready rinseability may be obtained by employing as a lubricant a concentrated aqueous solution of di-potassium phosphate or other highly water soluble inorganic salt that is capable of attaining a sufficient oily viscosity for lubricating 45 purposes. Such a solution may be prepared with a viscosity and lubricating character in the neighborhood of or slightly superior to the highly regarded lubricant, lard oil, and capable of competing in working qualities with this or other similar lubricating products. It is thus adapted to cold-working of metal with a benefit from its added desirable features. This particular material has a slight alkaline reaction which permits 50 it to combine with and neutralize traces of at-

mospheric carbonic acid which would otherwise facilitate metal corrosion.

Di-potassium phosphate is more satisfactory in certain ways than some other phosphates that approach it in desired qualifications in that it is somewhat hygroscopic and with concentrated solutions there is less tendency to crystallize. Moreover this tendency may be markedly restrained by addition of a suitable inhibiting agent. 5

The materials most nearly analogous in the physical properties mentioned are mono-sodium phosphate and mono-ammonium phosphate, since they are the most soluble of the ortho phosphates of the respective bases. They do have a slight 10 acid reaction, but the small amount of etching action that they may exert under ordinary conditions is not objectionable where painting, lacquering or enamelling constitute the final finish, nor is it undesirable on iron or steel where a final 15 phosphate coating is to be formed.

The sodium and ammonium phosphates are cheaper than di-potassium phosphate, and may be substituted in whole or in part for the potassium salt for purposes of economy, or where a 20 definite pH value is desired for any purpose, any such value between the alkaline value of the potassium salt and the acid value of the sodium or ammonium salt may be obtained by a proper mixture of the salts. 25

The efficiency as lubricants of the highly soluble and highly concentrated salts specified can be increased by addition of small quantities of a suitable wetting agent. For this purpose, among several available materials, I have preferred to 30 use sulphonated castor oil soap, since less than 1% dry basis by weight is sufficient to obtain the desired results, and it freely blends with the solution without foaming. Where the material is to be exposed in thin layers under drying con-

ditions that might result in objectionable evaporation, I have used additions of concentrated glycerine or diethylene glycol which have proved advantageous from this point of view and with the former material even up to amounts of 40 45 25% by volume. To attain highest viscosities, the glycerine has been added to the highly concentrated solution before cooling. Where an unusually highly bodied lubricant is desired, the concentration of the di-potassium phosphate may be carried to such an extent, before the addition of glycerine, that a finely divided suspended magma may result in the final solution. Such material as sulphonated castor oil soap may be used in addition to glycerine or the like in the 50 55

phosphate solution to decrease the drying or crystallizing tendencies without impairing the lubricating efficiency. Trouble from drying out may be avoided by the use of a thinner solution 5 where it will furnish the necessary lubrication.

The slight alkalinity of the di-potassium phosphate leaves the metal in a more rust-resistant condition than would a neutral or acid solution, and additional alkali may be added to the solution, or supplied in the rinse water when the 10 lubricant is removed, if it is desired with any of the solutions mentioned. Additional inhibition of rusting, after removal of the lubricant, may be secured by adding as little as .1% sodium bichromate or other chromate of an alkali metal.

In practice, since this new lubricating material can be washed off with clear water, I am able to readily recover the same, by use of a suitable counter current washing system that includes a slight amount of final concentration, for 20 reuse as lubricant or for other purposes. Where the heat of metal working produces sufficient evaporation, the lubricant solution direct from the counter current washing may be used as the 25 makeup solution for the lubricant. In any event the nature of the material is not changed by rinsing off, as is the character and availability of grease or oil when they are washed off with the aid of chemicals or soap.

30 The alkali phosphate lubricants mentioned above are particularly desirable when working metal that is to have formed on its surface a phosphate coat such as is widely used either as a finishing coat in itself or as a bond for such 35 a finishing coat as paint, lacquer or enamel.

Other inorganic salts have some of the characteristics of the phosphate salts mentioned, and might be used under some circumstances to a probably quite limited extent, but do not meet 40 the requirements so completely. For example, water glass or silicate of soda has a wide range of concentrations with appreciable viscosity and may be used as a lubricant under some conditions. An important disadvantage is that it acts 45 as an adhesive on drying and must be kept moist to be readily removable.

Under the same classification may be mentioned concentrated solutions such as zinc chloride or aluminum chloride, but for most common 50 metals they are of corrosive nature.

It will be understood that the cold working of the metal may be accomplished in any well known manner, and that the application of the coating for the final cold working may be by 55 any of the customary processes, this invention effecting no changes in these steps per se; yet the beneficial effects of the use of the new lubricant lie largely in the excellent and stable lubricating qualities combined with the ease and completeness of removal and the consequent uniformity and adhesion of the final finish coat applied.

Some alternatives have been described and specifically claimed, but it is understood that other 65 changes may be made within the scope of the appended claims.

What is claimed is:

1. The method which comprises coating metal with a concentrated aqueous solution of alkali 70 phosphate of the group consisting of dipotassium phosphate, mono-sodium phosphate and mono-ammonium phosphate, and cold working the metal while lubricated with said solution.

2. The method which consists in coating metal 75 with a concentrated solution of di-potassium

phosphate, and cold working the metal while lubricated with said solution.

3. The method which consists in coating metal with a concentrated solution of mono-sodium phosphate, and cold working the metal while 5 lubricated with said phosphate.

4. The method which consists in coating metal with a concentrated solution of mono-ammonium phosphate, and cold working the metal while coated with said phosphate.

5. The method which consists in coating metal with a concentrated aqueous solution of an alkali phosphate having a solubility in water of the order of that of di-potassium phosphate, cold-working the metal while so coated, washing the coating off of the formed metal, and applying a permanent protective coating to the washed surface.

6. The method which consists in coating a metal surface with a concentrated aqueous solution of a substantially non-corrosive, inorganic, 20 salt having a solubility in water of the order of that of di-potassium phosphate and containing a wetting agent, and cold-working the metal while lubricated by said solution.

7. The method which consists in coating a 25 metal surface with a concentrated aqueous solution of a substantially non-corrosive, inorganic salt having a solubility in water of the order of that of di-potassium phosphate and containing hygroscopic material, and cold-working the metal 30 while lubricated by said solution.

8. The method which consists in coating a metal surface with a concentrated aqueous solution of a substantially non-corrosive, inorganic salt having a solubility in water of the order of 35 that of di-potassium phosphate and containing a wetting agent and hygroscopic material, and cold-working the metal while lubricated by said solution.

9. The method which consists in coating metal 40 with a concentrated aqueous solution of an alkali phosphate having a solubility in water of the order of that of di-potassium phosphate and containing a wetting agent, and cold-working the metal while lubricated with said solution.

10. The method which consists in coating metal with a concentrated aqueous solution of an alkali phosphate having a solubility in water of the order of that of di-potassium phosphate and containing glycerine, and cold-working the metal 50 while lubricated with said solution.

11. The method which consists in coating metal with a concentrated aqueous solution of a substantially non-corrosive, inorganic salt having a solubility in water of the order of that of di-potassium phosphate containing a wetting agent, cold working the metal while lubricated with said solution, washing the solution from the shaped metal, and applying a permanent protective coating 55 to the washed surface.

12. The method which consists in coating metal with a concentrated aqueous solution of an alkali phosphate having a solubility in water of the order of that of di-potassium phosphate and containing a wetting agent, cold-working the metal 65 while lubricated with said solution, washing the solution from the shaped metal, and applying a permanent protective coating to the washed surface.

13. The method which consists in coating a 70 surface of iron or steel with a concentrated aqueous solution of an alkali phosphate having a solubility in water of the order of that of di-potassium phosphate, cold working the metal while lubricated with said solution, washing the solution 75

from the shaped surface, and applying a permanent rust-resisting coating to the washed surface.

14. A lubricating material comprising alkali phosphate of the group consisting of dipotassium phosphate, mono-sodium phosphate and mono-ammonium phosphate, and a wetting agent capable of reducing the surface tension of water.

15. A lubricating material comprising alkali phosphate of the group consisting of dipotassium phosphate, mono-sodium phosphate and mono-ammonium phosphate and hygroscopic material as hygroscopic as glycerine.

16. A lubricating material consisting of a concentrated solution of di-potassium phosphate

containing less than 1% of alkaline base sulphonated castor oil soap.

17. A lubricating material for metal consisting of a substantially non-corrosive inorganic salt having a solubility in water of the order of that of dipotassium phosphate and a wetting agent capable of reducing the surface tension of water.

18. A lubricating material consisting of a concentrated solution of di-potassium phosphate containing not over 1% of highly soluble sulphonated castor oil soap and not over 33% by volume of glycerine.

JOHN L. TUFTS.